# EUROPEAN PATENT SPECIFICATION

(11) **EP 3 483 337 B1**
(45) Date of publication and mention of the grant of the patent: **08.12.2021**
(21) Application number: 17306582.2
(22) Date of filing: 14.11.2017
(51) Int. Cl.: D21H 27/00, D21H 27/06, D21H 19/18, D21H 19/20, D21H 21/16

(54) **RECYCLABLE AND REPULPABLE TRANSLUCENT OR TRANSPARENT PAPER - USE FOR PACKAGING APPLICATIONS**
RECYCELBARES UND REPULPIERBARES TRANSLUZENTES ODER TRANSPARENTES PAPIER VERWENDUNG FÜR VERPACKUNGSANWENDUNGEN
PAPIER TRANSLUCIDE OU TRANSPARENT RECYCLABLE ET REPULPABLE À UTILISER POUR DES APPLICATIONS D'EMBALLAGE

(43) Date of publication of application: 15.05.2019
(73) Proprietor: AW BRANDING LIMITED, Aberdeen AB10 1HA (GB)
(72) Inventor: BAUMLIN, Jean-Marie, 62223 ANZIN SAINT-AUBIN (FR); DEPRES, Gaël, 38850 CHIRENS (FR); VAU, Jean-Marie, 75012 PARIS (FR); HARBURN-JONES, Glyn, Ashford,, Kent TN27 0BB (GB)
(74) Representative: Ernest Gutmann - Yves Plasseraud S.A.S.

(56) References cited:
- WO-A1-2014/080082
- WO-A2-2008/087337
- FR-A1- 2 883 570
- US-A- 4 271 227
- US-A- 5 006 389

## Description

### Field of the invention

The present invention relates to translucent or transparent paper suitable for laminate and packaging applications. More particularly, the present invention relates to a translucent paper having improved transparency by a coating process. Said transparent or translucent paper serves as a recyclable, repulpable and renewable alternative to plastic wrappers and laminates.

The invention also relates to a process for the manufacture of a transparent or translucent paper and to the use of the obtained paper in various domains including packaging of any type of goods such as consumer goods or food products.

The translucent or transparent paper of the invention comprises a fibrous substrate comprising cellulose fibers refined to above 40°SR and having an opacity less than or equal to 45 % measured in accordance with the ISO 2471 standard, preferably a natural tracing paper (i.e. tracing paper made of highly refined cellulose fibers), and a coating layer disposed (coated) on said fibrous substrate. Said coating layer enhances transparency of the fibrous substrate while also providing good barrier properties against moisture.

In one aspect, one or more coating layers are disposed on both the front side and the reverse side of the fibrous substrate. The coating layer(s) disposed on the front side and the reverse side of the fibrous substrate may or may not be of the same nature. The resulting translucent or transparent paper may be used as a wrapper for an item such as consumer goods or food products.

In another aspect, the reverse side of the fibrous substrate comprises a printed feature.

The printed feature is laterally inverted when viewed from the reverse side of the fibrous substrate and readable left-to-right when viewed from the front side of the fibrous substrate, through the coating layer(s) and the fibrous substrate. One or more layers of white ink may be disposed over the printed feature on the reverse side of the fibrous substrate in order to enhance contrast of the printed feature.

The present invention further discloses a product comprising said translucent or transparent paper, wherein said translucent or transparent paper is bonded, through a layer of glue or adhesive, to a paper or paperboard/cardboard support, for example in form of an item of any shape and size and accordingly, said translucent or transparent paper covers said support at least in part, for example its external surface or its internal surface, and possibly its entire surface.

The present invention also relates to a method of producing said translucent or transparent paper and a method of producing said product comprising said translucent or transparent paper.

Also disclosed is the use of said translucent or transparent paper for packaging, especially luxury packaging, in order to wrap, hold or laminate objects. Such packaging encompasses closed boxes or containers that protect, identify and transport a wide range of goods, including food and consumer products. The transparent or translucent paper of the invention may accordingly be provided in any format suitable for packaging such as sheets, or wrappers, which are flat, rolled, or folded. The paper of the invention accordingly acts as a protection of the element (whether liquid or solid) that it contacts, surrounds or contains, or as a cover which allows said element to be seen through the paper due to its transparency. In particular, the paper of the invention may serve the purpose of protecting the item it contacts, surrounds, contains or covers against scratches, fingerprints, oil/water stains, oxygen and other contaminants. In contrast to most packaging materials known in the art, the paper of the invention is not made of nor does it contain plastic film and may additionally have a soft surface that prevents abrasions and allows for color and touch effects.

### Background of the invention

Packaging materials such as wrappers are used to protect items against external aggressions and contaminants such as scratches, fingerprints, as well as oil and water stains. Petroleum-based plastics, in particular plastic films, are the most popular packaging material due to their low weight, flexibility, durability, transparency, versatility, as well as chemical stability.

Paper-plastic film laminates are also often used for packaging articles such as boxes and bags, especially for luxury goods.

Unfortunately, most plastics are currently made from non-renewable carbon sources and pose environmental concerns. In addition, they are not easily recycled. Thus, plastics do not provide a solution for companies looking for recyclability, environmental sustainability, and repulpability of packaging materials.

To this end, the two important actions necessary in the packaging industry are: first, using renewable raw materials, and second, facilitating recovery and recycling of used packaging materials.

The environmental concerns prompted the development and use of plastic films that are not derived from petroleum, such as PE films made from bioethanol. Although such plastic materials are renewable, it is difficult to recycle once they are laminated to paperboards.

There also exist plastics synthesized via green chemistry route. For example, plantbased polylactic acid (PLA) derived from corn starch, such as one developed by Toray, is gaining its popularity as an alternative to petroleum-derived plastics. This material is renewable and recyclable, but once it is laminated to a paperboard it is difficult to recycle.

European patent EP3087129 describes biodegradable plastics which are degradable into low molecular weight oligomers or monomers by the use of enzymes. Such plastics are recyclable but not necessarily renewable, and once laminated to a paperboard it is difficult to recycle.

US patent No. 4569888 teaches transparentized paper by means of impregnating polymers within the fibrous network and crosslinking in-situ. The process leads to highly transparentized paper which is recyclable and repulpable. However, the oil and gas barrier properties of the paper as well as the possibility of further enhancing transparency of such paper after the paper manufacturing process by simple means are not envisaged.

The inventors have advantageously designed a paper-based packaging material as an alternative to plastics used as wrappers or lamination films. Said paper-based packaging material is made from a renewable resource and is recyclable.

The paper of the invention accordingly solves the problem faced by the prior art that is to devise a recyclable and repulpable solution to replace packaging materials made of plastics, in particular plastic films. Further, the paper of the invention surprisingly affords delivering a transparent or translucent paper that has improved transparency compared to the known translucent paper, especially tracing paper, which also exhibits dimensional stability and barrier properties against external aggressions. In addition, such paper shows extra printability capabilities as it allows printing on the back face (or reverse side) of the paper alternatively or in addition to printing on the front face (or front side) when used. It may further have a tactile effect such as a soft-touch effect.

The physical structure of a paper allows for about 40 % light scattering from the top surface of the paper, about 20 % light scattering from the bulk of the paper, and about 40 % light scattering from the bottom surface of the paper, which add up to give 100 % opacity. Thus, by reducing the amount of light scattering, transparency is gained.

The invention discloses a paper sheet that is rendered more translucent or transparent than commonly known tracing papers. Up to 20 % of transparency may be gained (or up to 20 % of the light scattering ability is reduced) during the paper manufacturing process, for example by reducing the air/cellulose fiber interfaces or porosity within the bulk of the paper. Up to 40 % of transparency is gained by applying a coating on the top surface of the paper, and similarly, up to 40 % of transparency is gained by applying a coating (of the same or different nature from that of the top surface) on the bottom surface of the paper. The coating applied on the top or the bottom surface of the paper reduces the light scattering ability by reducing the surface irregularities and/or by reducing surface inhomogeneity present due to a refractive index mismatch between air bubbles and cellulose fibers. The present invention concerns transparentization by coating on the surface of a fibrous substrate, in particular translucent paper sheet, unlike transparentization that would take place by impregnation of said fibrous substrate. The coating layer accordingly does not substantially penetrate into the fibrous substrate, especially no deeper than filling in the surface irregularities/roughness of said fibrous substrate. Thus, the coating layer does not impregnate the fibrous substrate. In other words, the techniques applied to deposit the layer are conventional techniques leading to a short time scale of contact between the fibrous substrate and the coating composition before it starts to dry. This time scale is typically less than 10 seconds, or even less than 5 seconds.

The inventors have surprisingly observed that coating layer(s) may be defined and provided to reach enhanced transparency of a translucent paper used as substrate, in particular natural tracing paper, while creating moisture barrier property at the same time. In addition, the inventors have found that the addition of the moisture barrier property in the coating layer greatly reduced the hygro expansion coefficient of the translucent paper and consequently obtained an unexpected level of improvements in dimensional stability of said translucent or transparent paper, especially made from natural tracing paper with highly refined cellulose fibers. Furthermore, the transparentization of the translucent paper by applying coating layer(s) enabled a feature to be printed on the reverse side of the translucent of transparent in a reverse mode so that the printed feature is read from the front side of said translucent or transparent paper while being protected from moisture, oxygen, grease and other environmental factors.

The present invention is defined by the claims.

The invention advantageously may in addition to the disclosed properties above enable decreasing the roughness (Bendsten roughness) of the fibrous substrate when the coating layer has been applied on said substrate. This additional result may be obtained depending on the coating process which is used. As a result, the roughness of the coated face or faces may be less than 120 ml/mn, in particular may be in the range of about 70ml/mn.

Terms and phrases used in the present specification and in particular for the definition of the particular embodiments and the examples generally have meaning ordinary to those skilled in the art. In addition, the following terms are given the particular meaning as defined below. Such particular definition may be considered in combination with the ordinary meaning used by those skilled in the art.

The *"translucent or transparent paper"* of the present invention means a paper material or a paper object obtained from pulp fibers forming a fibrous substrate and is provided as a planar element, in particular a thin planar element such as a sheet of paper, having an opacity or transparency as disclosed herein, including in accordance with the particular embodiments of the Examples. The translucent or transparent paper of the present invention does not contain a plastic film, and thus is recyclable and/or repulpable. Other specific features of the transparent or translucent paper of the invention are disclosed herein.

The term *"opacity"* describes an extent to which an object, in particular a paper sheet, is seen through as some the light is not allowed to travel through the object. Opacity may be considered as inversely proportional to transparency. Opacity or transparency of a paper sheet can be measured by an apparatus known in the field, such as a spectrophotometer NOVICOLOR N5950.

The *"fibrous substrate"* as used herein refers to a material or object, in particular a sheet based on fibrous substrate, in particular a paper material or object, especially a paper sheet, and generally comprises vegetal fibers, cellulose fibers, in particular wood cellulose fibers, which are especially obtained from sustainable and environmentally friendly sources and processes. The fibrous substrate is advantageously translucent. Preferably, the fibrous substrate is a tracing paper, in particular natural tracing paper. Natural tracing paper derives its translucency primarily from the unusually high degree of refining given to the cellulose pulp fibers from which it is made. This results in a sheet without the air/fiber interfaces which give most papers their opacity. The translucency of natural tracing paper does not come from impregnation with an oil or other transparentizing chemical. The natural tracing paper may be a modified natural tracing paper that has improved folding endurance, greater resistance to tearing, greater stretch ability under tensile loading before a break occurs, reduced tensile strength and reduced stiffness, such as a urea-treated natural tracing paper as disclosed in European patent application EP1306484. Alternatives to a fibrous substrate consisting of tracing paper may encompass glassine paper, vellum paper, impregnated paper, and parchment paper or any paper substrate having basically transparent or translucent properties. Prepared tracing paper such as one treated with sulfuric acid may also be used as a translucent fibrous substrate.

According to the invention, at least one side of the fibrous substrate as defined above and in particular when it consists of a tracing paper is covered by a coating layer having a transparentization property and/or barrier properties including a moisture barrier property. The other side of the fibrous substrate may in particular be either a) bonded to a paper or paperboard item, b) printed with a feature before being bonded to a paper or paperboard item, or c) covered with same coating layer. In case of c), the resulting translucent or transparent paper may be used as a sheet, tape/strip/ribbon or wrapper or any other suitable format of a translucent or transparent paper that replaces plastic materials. The paper or paperboard item disclosed herein may comprise a printed feature, which may be covered (i.e. by bonding or lamination) by the transparent or translucent paper of the invention so that the printed feature is protected from moisture, grease and mechanical abrasion while visible through said transparent of translucent paper.

The terms *"repulpable paper"* and *"recyclable paper"* refer to the ability to reuse the paper as a raw material for producing a new paper. Different processes may be used to characterize this feature. Referred to herein is "*Voluntary standard for repulping and recycling corrugated fiberboard treated to improve its performance in the presence of water and water vapor"* as revised August 16, 2013.

The term *"coating layer"* refers to a dry or dried layer of material provided on at least the front side of the fibrous substrate by coating. The front side of the fibrous substrate is the side which faces the manufacturer of the user when displayed. The coating layer disposed on the front side of the fibrous substrate comprises a material that is suitable to provide barrier properties against moisture, oxygen and other gases when applied as a coating on the fibrous substrate. The coating layer is additionally regarded as a "transparentization layer" as the coating advantageously alleviates surface irregularities or roughness of the fibrous substrate, which significantly reduces the amount of light scattered off the surface of the fibrous substrate. The transparentizing property/function of the coating layer may also come from the reduced surface inhomogeneity present by refractive index mismatch between air bubbles and fibrous, in particular cellulose fibers. In such case, the refractive index of the coating layer is the same or very close to that of cellulose fibers thereby reducing the light scattering ability of the fibrous substrate. The coating layer may also penetrate within the fibrous substrate, thereby reducing any residual light scattering linked to the core/bulk of said fibrous substrate. The coating layer provided on the reverse side of the fibrous substrate may or may not be of the same nature but in any case serves the purpose of transparentizing the fibrous substrate in such a way described above. For example, an ink adhesion layer provided on the reverse side may be regarded as a coating layer of a different nature as long as it fulfills the purpose of transparentizing the fibrous substrate in such a way described above. Nevertheless, unless otherwise indicated, the coating layer provided on the reverse side of the fibrous substrate is of the same nature (i.e. same composition) as the coating layer provided on the front side of the fibrous substrate. Whenever the coating layer provided on the reverse side of the fibrous substrate is an ink adhesion layer having an ink adhesion property, it is clearly indicated so.

The coating layer may comprise a textured surface which is haptically perceptible. This can be achieved by the addition of chemicals which change the friction coefficient and/or particles which modify the roughness or the softness of the surface according to the rigidity and size of the particles.

The coating layer may comprise materials that are not necessarily renewable. In such case, the mass the non-renewable material comprised in the coating layer is very low relative to the total mass of the cellulose fibers in the translucent or transparent paper. This allows the translucent or transparent paper to be repulpable and/or recyclable.

The commercial products that can be used as coating layer include Epotal SP-106D from BASF (aqueous dispersion of Styrene 1,3-butadiene polymer), Galacryl 80.330.05 from Schmid Rhyner (Acrylic polymer), VaporCoat 2200 from Michelman ( Acrylic polymer), Evcote 3050 from Akzo Nobel (Water based polyester), SiOx deposition by vacuum deposition or Atomic Layer Deposition (such as Ceramis from Armcor, Chromatogenie from Centre Technique du papier Grenoble (fatty acid grafted on the paper by gas chemical reaction), MYSTOLENE PS from Catomance Technologies (paraffin wax and rosin), and AQUACER 497 from BYK Additives& Instruments (non-ionic aqueous emulsion of a paraffin wax).

Coating is performed according to any method well known in the art such as roll-to-roll coating, blade coating, spray coating, Mayer rod coating, air knife coating, direct gravure, offset gravure, reverse gravure, deep coating, smooth roll coating, curtain coating, bead coating, slot coating, twin HSM coating, film press coating, size press coating, transfer film method.

The term *"exposed face"* refers to either a face of the coating layer, the ink adhesion layer, the primer layer, the printed feature, or any other layer or deposit located opposite the fibrous substrate. The exposed face may in a particular embodiment be the front side of the translucent or transparent paper.

The term *"primer layer"* refers to a dry or dried layer of material optionally provided underneath the coating layer such that the primer layer is disposed or coated between the fibrous substrate and the coating layer in order to improve the spreadability of the coating composition that subsequently forms the coating layer when dried.

According to an embodiment of the invention, the optically transparent and electrically conductive material may be comprised within the coating layer (i.e. mixed in the coating layer composition) or may form a sub-layer of the coating layer.

The term *"sub-layer"* refers to a layer that is provided in conjunction with another layer. When the coating layer comprises a sub-layer of optically transparent and electrically conductive material, the sub-layer of optically transparent and electrically conductive material may be disposed on the outermost face of the coating layer (i.e. away from or opposite the fibrous substrate), beneath the coating layer (i.e. in contact with the fibrous substrate or the primer layer), or within the coating layer (i.e. buried in or surrounded by the coating layer).

The optically transparent and electrically conductive material is optionally disposed in conjunction with the coating layer and may form a continuous layer on a surface area from a few square millimeters up to tens of square centimeters. Such continuous layer may serve as an electrode in applications such as photovoltaics.

The optically transparent and electrically conductive material is optionally disposed in conjunction with the coating layer and may form one or more continuous traces having a width of microscopic scale, in particular a few micrometers, and a length in a range from a few micrometers up to a few centimeters or tens of centimeters. In particular it may be arranged as tracks. Said one or more continuous traces may serve as antenna(s) for RFID or NFC applications.

The layer or trace(s) of optically transparent and electrically conductive material may be formed by various coating or printing techniques known to those skilled in the art, which depend on the viscosity of such optically transparent and electrically conductive material provided or formulated by those skilled in the art.

The term *"ink adhesion layer"* refers to a layer that adheres an ink when a feature is required to be printed so that a desired printing quality can be met for various applications. The ink adhesion layer may alternatively be referred as "printable layer" or "ink adhesion promoter layer". The ink adhesion layer is advantageously transparent. Preferably, the ink adhesion layer also acts as a "transparentization layer" when applied on the reverse side of the fibrous substrate and alleviates surface irregularities or roughness of the fibrous substrate, which significantly reduces the amount of light scattered off the surface of the fibrous substrate. The ink adhesion layer may thus be regarded as a coating layer of different nature. The ink adhesion layer may have the same or very close refractive properties to that of cellulose fibers thereby reducing the light scattering ability of the fibrous substrate. The ink adhesion layer may also penetrate within the fibrous substrate, thereby reducing any residual light scattering linked to the core/bulk of said fibrous substrate.

The ink adhesion layer may be disposed directly on the reverse side of the fibrous substrate or on a coating layer provided on the reverse side of the fibrous substrate.

The *"printed feature"* refers to any image or text printed in color or black and white, using various printing techniques including, but not limited to offset printing, inkjet printing, laser printing, xerographic printing, screen printing, flexographic printing, continuous inkjet, liquid toner printing, letterpress, laser engraving, hot foil blocking.

The printed feature may be disposed on the reverse side of the fibrous substrate in various modes: (a) directly on the fibrous substrate, (b) on a coating layer that is disposed on the fibrous substrate or on a primer layer, or (c) on an ink adhesion layer that is disposed on the fibrous substrate or on a coating layer.

The printed feature is advantageously printed in a reverse or mirror mode (i.e. left/right reversal) so that the printed feature can be readable from the front side of the transparentized fibrous substrate or of translucent or transparent paper.

By printing on the reverse side of the fibrous substrate, it makes it possible that the printed feature is protected from any external factors such as moisture, oxygen, grease and scratches.

The" *white ink'* is advantageously disposed on the printed feature so as to cover the printed feature and preferably disposed on the entirety of the reverse side of the fibrous substrate. The white ink increases contrast of the printed feature, which is viewed from the front side of the fibrous substrate or of translucent or transparent paper.

The invention also relates to a product that comprises the translucent or transparent paper according to the invention bonded by any available technique in particular laminated to a paper or paperboard item, such as folded paper box, and assembled box or case made from hard paperboard or a bag made of paper, paperboard or cardboard.

The translucent of transparent paper of the invention may be bonded to a standard paper, cardboard or paperboard (generally designated as a paper support) printed with a feature through a layer of glue or adhesive disposed in between the two.

The glue, which may be referred as an adhesive is used to bond the translucent or transparent paper of the invention, which may or may not comprise a printed feature on the reverse side of the fibrous substrate, to any paper or paperboard items.

The glue or adhesive is preferably transparent or white and applied in a continuous layer so as to ensure that no air bubbles or gaps are created between the translucent or transparent paper and the item or the object to which said translucent or transparent paper is adhered. The glue or adhesive advantageously has good moisture barrier property.

Additional features and details appear in the Examples which follow and in the figure. Throughout the examples, natural tracing paper was used to demonstrate specific embodiments of the invention.

Figure 1 discloses the hygroexpansivity of coated tracing paper of Example 6 measured by a Varidim apparatus.

### Examples

Example 1: A sheet of coated paper having a basis weight of 115 g/m² (obtained from Satimat) was printed by xerography in black, and a tracing paper was bonded against the printing with solvent-based two-component polyurethane adhesive containing ADCOTE 548-81R (from DOW EUROPE GmbH) and Ethyl Acetate. The brightness was measured with a spectrophotometer NOVICOLOR N5950under ISO 2469 through the tracing paper before and after the application of a coating layer by a Meyer rod. The Epotal SP-106D is an anionic dispersion of a styrene-butadiene copolymer, which provide a moisture barrier property. The Galacryl 80.330.05 is an acrylic glossy varnish. The Diofan A297 is an aqueous emulsion of polyvinylidene chloride. The obtained values are as follows:

| grammage (g/m²) | layer | Coat weight (g/m²) | Brightness before coating | Brightness after coating |
|---|---|---|---|---|
| 42 | DIOFAN A 297 | 9,4 | 9,2 | 7,7 |
| 42 | EPOTAL | 6,8 | 9,9 | 9,4 |
| 42 | GALACRYL 80.330.05 | 8,2 | 7,8 | 4,6 |
| 62 | DIOFAN A 297 | 7,6 | 9,3 | 8,1 |
| 62 | EPOTAL | 6,2 | 10,4 | 10,6 |
| 62 | GALACRYL 80.330.05 | 7,0 | 10,8 | 8,4 |
| 102 | EPOTAL | 6,3 | 12,2 | 12,3 |
| 102 | GALACRYL 80.330.05 | 7,3 | 10,0 | 7,1 |

The lower the brightness was, the darker was the shade through the tracing paper. It was observed that the thinner the tracing paper was, the lower the brightness was. The brightness was lower after coating except the coating with Epotal. Galacryl 80.330.05 and Diofan A297 improved the visibility of the printed feature.

Example 2: Three sheets of tracing paper sheets, each having a basis weight of 82 g/m², 112 g/m² and 180g/m², were printed by a four-color offset printing press Sakurai LED UV and covered by a white print applied by screen printing. The inks used were Xcura Black, Cyan, Magenta, and Yellow. The 100% ink coverage had ink densities between 1.2 and 1.5 for black, 1 and 1.1 for cyan, 0.9 and 1 for magenta and 0.8 and 0.9 for yellow. A transparentization layer was coated on the non-printed side by Meyer rod coating. The brightness measured on the 100% black print through the paper is as follows:

| Translucent 82 gsm | | Offset |
|---|---|---|
| material | Coat Weight (g/m²) | Brightness |
| no layer | 0 | 8.5 |
| Diofan A 297 | 6.2 | 8 |
| Diofan A 297 | 11.8 | 5.9 |
| Epotal SP-106 D | 3.2 | 7.9 |
| Epotal SP-106 D | 7.1 | 7.6 |
| Epotal SP-106 D | 10 | 7 |

| Translucent 112 gsm | | Offset |
|---|---|---|
| material | Coat Weight (g/m²) | Brightness |
| no layer | 0 | 11.8 |
| Diofan A 297 | 7.9 | 9.2 |
| Diofan A 297 | 13.1 | 8.7 |
| Epotal SP-106 D | 7.4 | 9.8 |
| Epotal SP-106 D | 11.2 | 9.4 |

The inventors observed that the brightness of solid black measured above was reduced when one of the coating layer compositions Diofan A297 or Epotal SP-103 D was applied. The printed feature was visually distinct through the tracing paper. The best result was obtained with the thinnest (i.e. having the lowest basis weight) tracing paper.

Example 3: The two sides of tracing paper sheets, each having a basis weight of 112 g/m² and 180 g/m², were applied with an adhesion promoter for liquid toner ink. These sheets were printed by liquid toner using HP Indigo 7800 press. The image formed by 4 colors was covered by two layers of 100 % white ink. The non-printed side was coated with a transparentization layer by Meyer rod coating. The brightness measured on the 100 % black print is as follows:

| Translucent 112 gsm | | liquid Toner |
|---|---|---|
| material | Coat Weight (g/m²) | Brightness |
| no layer | 0 | 11.6 |
| Diofan A 297 | 5.2 | 10.6 |
| Diofan A 297 | 10.6 | 9.7 |
| Epotal SP-106 D | 5.5 | 11.2 |
| Epotal SP-106 D | 11.2 | 10.1 |
| Galacryl 80,330,05 | 4.7 | 9.8 |
| Galacryl 80,330,05 | 9 | 8.4 |

| Translucent 180 gsm | | liquid Toner |
|---|---|---|
| material | Coat Weight (g/m²) | Brightness |
| no layer | 0 | 11.7 |
| Diofan A 297 | 6.4 | 11.2 |
| Diofan A 297 | 11.4 | 9.9 |

Example 4: A coating was applied on a side of a tracing paper having a basis weight of 52 g/m² using a Mayer rod. On the one hand, a product Galacryl 80.330.05 was applied at a rate of 11.3 g/m²/sec. On the other hand, 12.9 g/m² of a product Diofan A297 was applied. The water vapor transmission rate was achieved in accordance with the test method ISO 2528 under which the sample was placed at 23°C with an atmosphere of 85% RH on one side and a desiccant on the other.

| | Water vapor transmission rate (g/m²/day) | Opacity index |
|---|---|---|
| Tracing paper only | 23.7 | 28.8 |
| With a layer of Galacryl 80.330.05 | 15.3 | 17.8 |
| With a layer of Diofan A297 | 3.3 | 18.9 |

Example 5: A coating of Diofan A297 (from Solvay) was deposited in a different amount between 8 and 22 g/m² on both sides of a tracing paper having a basis weight of 62 g/m² (from Arjowiggins). The drying was carried out at 120 °C. The table below shows the opacity index of the sheets.

| Sample | Coat Weight (g/m²) | Opacity index |
|---|---|---|
| Tracing paper only | - | 25.3 |
| coating Diofan A 297 | 8.5 | 17 |
| coating Diofan A 297 | 10 | 17 |
| coating Diofan A 297 | 12 | 14.5 |
| coating Diofan A 297 | 14 | 16.5 |
| coating Diofan A 297 | 21 | 11.7 |

Example 6: The table below shows hygroexpansivity of two tracing papers having a basis weight of 62 g/m², each coated with Diofan A 297 with a coat weight of 10 g/m² and 12 g/m². The hygroexpansivity/dimensional variations (measured along the crossgrain direction) was obtained by using a Varidim apparatus, which measured the variation of dimensions in function of different humidity cycles.

| | Varidim | | | | | | | | | | | | |
|---|---|---|---|---|---|---|---|---|---|---|---|---|---|
| | Relative length variation (%) | | | | | | | | | | | | |
| **Relative Humidity** | **RH 50** | **RH 80** | **RH 50** | **RH 15** | **RH 50** | **RH 80** | **RH 50** | **RH 15** | **RH 50** | **RH 80** | **RH 50** | **RH 15** | **RH 50** |
| **Tracing 62 g/m²** | 0 | 1.25 | 0.08 | -1.04 | -0.24 | 1.1 | 0 | -1.12 | -0.31 | 1.02 | -0.06 | -1.16 | -0.35 |
| **Diofan A297 10 g/m²** | 0 | 0.4 | 0.31 | 0.13 | 0.13 | 0.48 | 0.35 | 0.16 | 0.16 | 0.5 | 0.36 | 0.16 | 0.16 |
| **Diofan A297 12 g/m²** | 0 | 0.15 | 0.13 | 0.03 | 0.03 | 0.16 | 0.13 | 0.02 | 0.03 | 0.16 | 0.12 | 0.05 | 0.05 |

For the standard tracing paper, the peak-to-peak variations are 2.3 % (1.25 + 1.09 for example for the two first peaks) while for the tracing paper coated with Diafan rod 16M, the peak-to-peak variations are only 0.12 % (0.15 - 0.03), which corresponds to a dimensional variation reduced by a factor of 19.

Example 7: A coating of Diofan A297 was applied on a side of three tracing papers, each having a basis weight of 42 g/m², 102 g/m**²** and 140g/m², using a Meyer rod. The resulting opacity is summarized as follows:

| Translucent 42 gsm | | | | |
|---|---|---|---|---|
| material | Coat Weight (front side (g/m²) | Opacity | Coat Weight (reverse side) (g/m²) | Opacity |
| no layer | 0 | 25.8 | | |
| Diofan A 297 | 5.3 | 21.9 | 7.2 | 17.9 |
| Diofan A 297 | 11.3 | 19.7 | 10.9 | 17 |

| Translucent 102 gsm | | Translucent 102 gsm | | |
|---|---|---|---|---|
| material | Coat Weight (g/m²) | Opacity | | |
| no layer | 0 | 32.3 | | |
| Diofan A 297 | 7.1 | 28.7 | | |
| Diofan A 297 | 11.5 | 27.6 | | |

| Translucent 140 gsm | | | | |
|---|---|---|---|---|
| material | Coat Weight (g/m²) | Opacity | | |
| no layer | 0 | 42.6 | | |
| Diofan A 297 | 9 | 39.7 | | |
| Diofan A 297 | 14.1 | 38.5 | | |

The inventors observed that the thinner the tracing paper was, the less opaque was the resulting paper. The thicker the coating layer was, the greater was the decrease in opacity.

The inventors surprisingly observed a very sharp decline in the opacity that exceeded their expectations, as they managed to decrease the opacity by a factor of 2.2.

Example 8: The tracing paper possesses the following characteristics:

| measure | method | Unit | value |
|---|---|---|---|
| Grammage | ISO 536 | g/m² | 63.5 |
| Caliper | ISO 534 | µm | 56.0 |
| Moisture | ISO 287 | % | 7.8 |
| Tear MD | ISO 1974 | daN | 144 |
| Tear CD | ISO 1974 | daN | 176 |
| Contrast Ratio | ISO 2469 | | 18.1 |
| Whiteness | ISO 5631-2 | | 56.5 |
| Colour L | ISO 5631-2 | | 85.4 |
| a | ISO 5631-2 | | -0.5 |
| b | ISO 5631-2 | | 2.0 |
| Burst | ISO 2758 | kPa | 272 |
| Fold MD | ISO 5626 | | 2085 |
| Fold CD | ISO 5626 | | 826 |
| Surface pH | TAPPI 5290M / ISO 6588 | | 6.6 |
| Stiffness MD | ISO 2493-2 | mN | 22.9 |
| Stiffness CD | ISO 2493-2 | mN | 8.9 |
| Roughness Top | ISO 8791-2 | mL/mn | 115 |
| Roughness Back | ISO 8791-2 | mL/mn | 101 |

The water vapor transmission rate achieved in accordance with the test method TAPPI/ANSI T 464 om-12 under which the sample to test was place at 37.8°C with an atmosphere of 90% RH on one side and a desiccant on the other was 96.5 g/m²/day at. The opacity was 26 %.

The tracing paper was coated on a reel by smooth roll coating method. The coating layer was applied on both sides (the front side and the reverse side) with an amount of 4g/m² per side.

When the applied coating layer was a protection varnish, the water vapor transmission rate was 47.1 g/m²/day. The opacity was 20.2 %.

When the applied coating layer was a dried aqueous emulsion of polyvinylidene chloride (PVDC), the water vapor transmission rate was 16.8 g/m²/day. The opacity was 24.4 % and the tracing paper was repulpable.

## Claims

1. A translucent or transparent paper comprising:
(i) a fibrous substrate having a front side and a reverse side, the fibrous substrate comprising cellulose fibers refined to above 40 °SR and the opacity index of said fibrous substrate being less than or equal to 45 % measured in accordance with the ISO 2471 standard; and
(ii) one or more coating layers, in particular one or two coating layers disposed on the front side of said fibrous substrate, comprising a material chosen from material conferring moisture barrier properties and having transparentization capability when provided as a coating layer on said fibrous substrate and enabling the translucent or transparent paper to be repulpable, said material being chosen from the group comprising or consisting of copolymer or homopolymer of vinylidene chloride, copolymer or homopolymer of styrene such as styrene 1,3-butadiene polymer, copolymer or homopolymer of acrylic, copolymer or homopolymer of polyester, or paraffin such as paraffin wax.

2. The translucent or transparent paper of claim 1 wherein one or more coating layers are also disposed on the reverse side of the fibrous substrate

3. The translucent or transparent paper of claim 1 or 2 having at least one of the following features or combination thereof: (i) a hygroexpansivity less than or equal to 1 %, preferably less than or equal to 0.5 %, and even more preferably less or equal to 0.25%, when changing Relative Humidity (RH) from 15% to 80% then to 15% in 8 hours, or (ii) a water vapor transmission rate less than or equal to 20 g/m²/day at 85 % of differential RH and 23 °C, or less than or equal to 10 g/m²/day at 85 % of differential RH and 23 °C, or less than or equal to 5 g/m²/day at 85 % of differential RH and 23 °C.

4. The translucent or transparent paper of any of claims 1 to 3 having an opacity index less than or equal to 20 % measured in accordance with the ISO 2471 standard.

5. The translucent or transparent paper of any of claims 1 to 4, wherein the fibrous substrate has a basis weight in a range from 40 to 200 g/m2, in particular in a range from 40 to 140 g/m², and preferably in a range from 40 to 90 g/m².

6. The translucent or transparent paper of any of claims 1 to 5, wherein the fibrous substrate comprises cellulose fibers refined to 60 °SR or above 80 °SR.

7. The translucent or transparent paper of any of claims 1 to 6, wherein the fibrous substrate is a tracing paper.

8. The translucent or transparent paper of any of claims 1 to 7, wherein the total coating layer(s) on one side of the fibrous substrate has a dry coat weight in a range from 1 to 40 g/m², preferably from 2 to 20 g/m², even more preferably from 4 to 12 g/m².

9. The translucent or transparent paper of any of claims 1 to 8, wherein at least one coating layer comprises a copolymer or homopolymer of vinylidene chloride, in particular a dried latex film of copolymer of vinylidene chloride or homopolymer of vinylidene chloride (PVDC).

10. The translucent or transparent paper of any of claims 1 to 9, wherein an ink adhesion layer is disposed on the reverse side of the fibrous substrate in the absence of a coating layer or an ink adhesion layer is disposed on the exposed face of the coating layer(s) that is/are provided on the reverse side of the fibrous substrate, the ink adhesion layer having a thickness in a range from 0.1 to 4 µm, in particular an ink adhesion layer comprising any of styrene acrylate, styrene butadiene, polyvinyl acetate, polyethylene acrylic acid, or modified starch, or a combination thereof.

11. The translucent or transparent paper of any of claims 1 to 10, wherein at least a portion of the exposed face of the ink adhesion layer or the exposed face of the coating layer disposed on the reverse side of the fibrous substrate comprises a printed feature, which is laterally inverted so that the feature is readable from the exposed face of the coating layer disposed on the front side of the fibrous substrate and through the fibrous substrate.

12. The translucent or transparent paper of claim 11, wherein one or more layers of white ink are disposed on the printed feature or the entirety of the reverse side of the fibrous substrate comprising said printed feature.

13. A product comprising a translucent or transparent paper according to any of claims 1 to 12, wherein the translucent or transparent paper is bonded to a paper, cardboard or paperboard item, with a layer of glue or adhesive disposed between said paper, cardboard or paperboard item and the coating layer(s) or the printed feature or the white ink layer(s) on the reverse side of the fibrous substrate, said glue or adhesive having a thickness in a range from 2 to 12 µm, in particular a glue or adhesive comprising a material selected from polyurethane adhesives, acrylic adhesives, one or two-component polychloroprene adhesive, polyvinyl acetate, modified starch, methylcellulose, vinylic dispersion.

14. A process for producing a translucent or transparent paper according to any of claims 1 to 13, comprising:
a) providing or producing a fibrous substrate having a front side and a reverse side, wherein the fibrous substrate comprising cellulose fibers refined to above 40 °SR and the opacity index of said fibrous substrate is less than or equal to 45 % measured in accordance with the ISO 2471 standard;
b) applying a coating composition on the front side of the fibrous substrate, the coating composition comprising a material chosen from material conferring moisture barrier properties and having transparentization capability when provided as a coating layer on said fibrous substrate and enabling the translucent or transparent paper to be repulpable, said material being chosen from the group comprising or consisting of copolymer or homopolymer of vinylidene chloride, such as aqueous dispersion of said copolymer or comopolymer of vinylidene chloride, copolymer or homopolymer of styrene such as aqueous dispersion of copolymer or homopolymer of styrene, such as styrene 1,3-butadiene, copolymer or homopolymer of acrylic, copolymer of homopolymer of polyester, in particular water-based polyester, or paraffin such as paraffin wax;
c) drying the coating composition at a temperature between 70 and 200 °C for 0.2 to 1 minute, so as to form a coating layer having a thickness in a range from 1 to 40 µm, preferably from 2 to 20 µm, even more preferably from 4 to 12 µm;
d) optionally repeating steps b) and c) at least once; and
e) optionally also applying and drying said coating composition on the reverse side of the fibrous substrate at least once, and/or applying and drying a composition for an ink adhesion layer on the reverse side of the fibrous substrate or on the coating layer(s) disposed on the reverse side,
in particular wherein said coating composition and a composition for a ink adhesion layer are applied by a technique selected from roll-to-roll coating, blade coating, spray coating, Mayer rod coating, air knife coating, direct gravure, offset gravure, reverse gravure, deep coating, smooth roll coating, curtain coating, bead coating, slot coating, twin HSM coating, film press coating, size press coating, and/or transfer film method, in particular air knife coating or reverse gravure coating.

15. The process of claim 14, wherein a feature is printed on the exposed face of the ink adhesion layer or the exposed face of the coating layer disposed on the reverse side of the fibrous substrate in reverse or mirror mode (i.e. left/right reversal) by a technique selected from offset printing, inkjet printing, laser printing, xerographic printing, screen printing, flexographic printing, continuous inkjet, liquid toner printing, letterpress, laser engraving, and/or hot foil blocking, in particular offset printing, inkjet printing, screen printing, continuous inkjet, liquid toner printing.

16. The process of claim 15, wherein one or more layers of white ink are applied over the printed feature by a technique selected from roll-to-roll coating, blade coating, spray coating, Mayer rod coating, air knife coating, direct gravure, offset gravure, reverse gravure, deep coating, smooth roll coating, curtain coating, bead coating, slot coating, twin HSM coating, film press coating, size press coating, transfer film method, offset printing, inkjet printing, laser printing, xerographic printing, screen printing, flexographic printing, continuous inkjet, liquid toner printing, hot foil blocking, especially by screen printing, liquid toner printing, and offset printing.

17. A process for producing a product of claim 13 comprising carrying out the steps of the process according to claims 14 to 16, wherein in addition, a layer of glue is applied on the coating layer or on the white ink layer and/or a surface of a paper, cardboard or paperboard item so as to bond the translucent or transparent paper and the paper, cardboard or paperboard item.

18. The use of the translucent or transparent paper of claims 1 to 17 for packaging, especially luxury packaging, as a transparent or translucent protective ribbon, pocket, wrapper, or a plastic laminate replacement/alternative wherein optionally the packaging is heat sealed when the coating layer of the paper comprises a copolymer or homopolymer of vinylidene chloride in particular homopolymer of vinylidene chloride (PVDC).

## Patentansprüche

1. Transluzentes oder transparentes Papier, umfassend:
(i) ein faseriges Substrat mit einer Vorderseite und einer Rückseite, wobei das faserige Substrat Zellulosefasern umfasst, die auf mehr als 40 °SR raffiniert sind, und wobei der Opazitätsindex des genannten faserigen Substrats niedriger als oder gleich 45 % gemessen gemäß der ISO-Norm 2471 ist; und
(ii) eine oder mehrere Beschichtungsschicht(en), insbesondere eine oder zwei Beschichtungsschicht(en), die auf der vorderen Seite des genannten faserigen Substrats angeordnet ist/sind, umfassend ein Material, das aus Material ausgewählt ist, das Feuchtigkeitssperre-Eigenschaften verleiht und eine Fähigkeit zum Transparentmachen aufweist, wenn sie als eine Beschichtungsschicht auf dem genannten faserigen Substrat bereitgestellt ist und es dem transluzenten oder transparenten Papier ermöglicht, einstampfbar zu sein, wobei das genannte Material aus der Gruppe gewählt ist, umfassend oder bestehend aus Vinylidenchlorid-Kopolymer oder -Homopolymer, Styrol-Kopolymer oder -Homopolymer, wie z. B. Styrol-1,3-Butadienpolymer, Acryl-Kopolymer oder-Homopolymer, Polyester-Kopolymer oder -Homopolymer, oder Paraffin, wie z. B. Paraffinwachs.

2. Transluzentes oder transparentes Papier gemäß Anspruch 1, wobei eine oder mehrere Beschichtungsschicht(en) ebenfalls auf der Rückseite des faserigen Substrats angeordnet ist/sind.

3. Transluzentes oder transparentes Papier gemäß Anspruch 1 oder 2 mit wenigstens einem der folgenden Merkmale oder einer Kombination davon: (i) eine Feuchtdehnung von weniger als oder gleich 1 %, bevorzugt weniger als oder gleich 0,5 % und weiter bevorzugt weniger als oder gleich 0,25%, beim Ändern der Relativen Feuchtigkeit (RH) von 15 % auf 80 %, dann von 15 % in 8 Stunden oder (ii) eine WasserdampfÜbertragungsrate von weniger als oder gleich 20 g/m²/Tag bei 85 % einer Differenzial-RH und 23 °C oder weniger als oder gleich 10 g/m²/Tag bei 85 % einer Differenzial-RH und 23 °C oder weniger als oder gleich 5 g/m²/Tag bei 85 % bei einer Differenzial-RH und 23 °C.

4. Transluzentes oder transparentes Papier gemäß irgendeinem der Ansprüche 1 bis 3 mit einem Opazitätsindex von weniger als oder gleich 20 %, gemessen gemäß der ISO-Norm 2471.

5. Transluzentes oder transparentes Papier gemäß irgendeinem der Ansprüche 1 bis 4, wobei das faserige Substrat ein Basisgewicht in einem Bereich von 40 bis 200 g/m2, insbesondere in einem Bereich von 40 bis 140 g/m² und bevorzugt in einem Bereich von 40 bis 90 g/m² aufweist.

6. Transluzentes oder transparentes Papier gemäß irgendeinem der Ansprüche 1 bis 5, wobei das faserige Substrat bis auf 60 °SR oder von mehr als 80 °SR raffinierte Zellulosefasern umfasst.

7. Transluzentes oder transparentes Papier gemäß irgendeinem der Ansprüche 1 bis 6, wobei das faserige Substrat ein Pauspapier ist.

8. Transluzentes oder transparentes Papier gemäß irgendeinem der Ansprüche 1 bis 7, wobei die gesamte(n) Beschichtungsschicht(en) auf einer Seite des faserigen Substrats ein Trockenschichtgewicht in einem Bereich von 1 bis 40 g/m², bevorzugt von 2 bis 20 g/m², weiter bevorzugt von 4 bis 12 g/m² aufweist/aufweisen.

9. Transluzentes oder transparentes Papier gemäß irgendeinem der Ansprüche 1 bis 8, wobei wenigstens eine Beschichtungsschicht ein Vinylidenchlorid-Kopolymer oder - Homopolymer, insbesondere einen getrockneten Latexfilm aus Vinylidenchlorid-Kopolymer oder -Homopolymer (PVDC) umfasst.

10. Transluzentes oder transparentes Papier gemäß irgendeinem der Ansprüche 1 bis 9, wobei bei Fehlen einer Beschichtungsschicht eine Druckfarben-Anhaftschicht auf der Rückseite des faserigen Substrats angeordnet ist oder eine Druckfarben-Anhaftschicht auf der freigelegten Seite der Beschichtungsschicht(en) angeordnet ist, die auf der Rückseite des faserigen Substrats bereitgestellt ist/sind, wobei die Druckfarben-Anhaftschicht eine Dicke in einem Bereich von 0,1 bis 4 pm, insbesondere eine Druckfarben-Anhaftschicht aufweist, umfassend Styrolacrylat, Styrolbutadien, Polyvinylacetat, Polyethylenacrylsäure oder modifizierte Stärke oder eine Kombination davon.

11. Transluzentes oder transparentes Papier gemäß irgendeinem der Ansprüche 1 bis 10, wobei wenigstens ein Abschnitt der freigelegten Seite der Druckfarben-Anhaftschicht oder der freigelegten Seite der Beschichtungsschicht, die auf der Rückseite des faserigen Substrats angeordnet ist, ein bedrucktes Merkmal umfasst, das derart seitlich umgekehrt ist, dass das Merkmal von der freigelegten Seite der Beschichtungsschicht, die auf der Vorderseite des faserigen Substrats angeordnet ist, und durch das faserige Substrat lesbar ist.

12. Transluzentes oder transparentes Papier gemäß Anspruch 11, wobei eine oder mehrere Schicht(en) aus weißer Druckfarbe auf dem bedruckten Merkmal oder der Gesamtheit der Rückseite des faserigen Substrats, umfassend das genannte bedruckte Merkmal, angeordnet ist/sind.

13. Produkt, umfassend ein transluzentes oder transparentes Papier gemäß irgendeinem der Ansprüche 1 bis 12, wobei das transluzente oder transparente Papier an einem Papier-, Karton- oder Pappartikel mit einer zwischen dem genannten Papier-, Karton- oder Pappartikel und der Beschichtungsschicht(en) oder dem bedruckten Merkmal oder der/den weißen Druckfarben-Schicht(en) auf der Rückseite des faserigen Substrats angeordneten Schicht aus Klebstoff oder Haftmittel aufgeklebt ist, wobei der genannte Klebstoff oder das genannte Haftmittel eine Dicke in einem Bereich von 2 bis 12 pm aufweist, wobei insbesondere ein Klebstoff oder ein Haftmittel ein Material umfasst, das aus Polyurethan-Haftmitteln, Acryl-Haftmitteln, Einem- oder Zwei-Komponenten-Polychoroprenhaftmittel, Polyvinylacetat, modifizierter Stärke, Methylzellulose, Vinyldispersion ausgewählt ist.

14. Verfahren zum Produzieren eines transluzenten oder transparenten Papiers gemäß irgendeinem der Ansprüche 1 bis 13, umfassend:
a) Bereitstellen oder Produzieren eines faserigen Substrats mit einer Vorderseite und einer Rückseite, wobei das faserige Substrat Zellulosefasern umfasst, die auf mehr als 40 °SR raffiniert sind, und wobei der Opazitätsindex des genannten faserigen Substrats niedriger als oder gleich 45 %, gemessen gemäß der ISO-Norm 2471 ist;
b) Anwenden einer Beschichtungszusammensetzung auf der Vorderseite des faserigen Substrats, wobei die Beschichtungszusammensetzung ein Material umfasst, das aus Material ausgewählt ist, das Feuchtigkeitssperre-Eigenschaften verleiht und eine Fähigkeit zum Transparentmachen aufweist, wenn sie als eine Beschichtungsschicht auf dem genannten faserigen Substrat bereitgestellt ist und es dem transluzenten oder transparenten Papier ermöglicht, einstampfbar zu sein, wobei das genannte Material aus der Gruppe gewählt ist, umfassend oder bestehend aus Vinylidenchlorid-Kopolymer oder -Homopolymer, wie z. B. eine wässerige Dispersion aus dem genannten Vinylidenchlorid-Kopolymer oder -Homopolymer, Styrol-Kopolymer oder - Homopolymer, wie z. B eine wässerige Dispersion aus Styrol-Kopolymer oder -Styrol, wie z. B. Styrol-1,3-Butadienpolymer, Acryl-Kopolymer oder -Homopolymer, Polyester-Kopolymer oder - Homopolymer, insbesondere wasserbasiertes Polyester, oder Paraffin, wie z. B. Paraffinwachs;
c) Trocknen der Beschichtungszusammensetzung bei einer Temperatur zwischen 70 und 200 °C über 0,2 bis 1 Minute derart, dass eine Beschichtungsschicht mit einer Dicke in einem Bereich von 1 bis 40 pm, bevorzugt von 2 bis 20 pm, weiter bevorzugt von 4 bis 12 pm gebildet ist;
d) Optional Wiederholen der Schritte b) und c) wenigstens einmal; und
e) optional ebenfalls Anwenden und Trocknen der genannten Beschichtungszusammensetzung auf der Rückseite des faserigen Substrats wenigstens einmal und/oder Anwenden und Trocknen einer Zusammensetzung für eine Druckfarben-Anhaftschicht auf der Rückseite des faserigen Substrats oder auf der/den auf der Rückseite angeordneten Beschichtungsschicht(en),
wobei insbesondere die genannte Beschichtungszusammensetzung und eine Zusammensetzung für eine Druckfarben-Anhaftschicht durch eine Technik angewendet sind, die aus Rolle-zu-Rolle-Beschichtung, Rakelbeschichtung, Sprühbeschichtung, Mayer-Bar-Beschichtung, Luftpinselbeschichtung, direkter Gravur, Offset-Gravur, Umkehrgravur, Tiefenbeschichtung, Weichrollenbeschichtung, Gießverleimung, Schwallbeschichtung, Schlitzbeschichtung, Zwillings-HSM-Beschichtung, Filmpressenbeschichtung, Größenpressenbeschichtung und/oder Übertragungsfilmverfahren, insbesondere Luftpinselbeschichten oder Umkehrgravurbeschichtung ausgewählt ist.

15. Verfahren gemäß Anspruch 14, wobei ein Merkmal auf der freigelegten Seite der Druckfarben-Anhaftschicht oder der freigelegten Seite der Beschichtungsschicht aufgedruckt ist, die auf der Rückseite des faserigen Substrats im Umkehr- oder Spiegelmodus (d. h. Links-/Rechts-Umkehrung) durch eine Technik angeordnet ist, die aus Offset-Drucken, Tintenstrahldrucken, Laserdrucken, xerographischem Drucken, Rasterdrucken, flexographischem Drucken, kontinuierlichem Tintenstrahl, Füssugtoner-Drucken, Buchdruck, Lasergravur und/oder Heißfolienblockieren, insbesondere Offset-Drucken, Tintenstrahldrucken, Rasterdrucken, kontinuierlichem Tintenstrahl, Flüssigtoner-Drucken ausgewählt ist.

16. Verfahren gemäß Anspruch 15, wobei eine oder mehrere Schicht(en) aus weißer Druckfarbe über dem bedruckten Merkmal durch eine Technik angewendet ist/sind, die aus Rolle-zu-Rolle-Beschichtung, Rakelbeschichtung, Sprühbeschichtung, Mayer-Bar-Beschichtung, Luftpinselbeschichtung, direkter Gravur, Offset-Gravur, Umkehrgravur, Tiefenbeschichtung, Weichrollenbeschichtung, Gießverleimung, Schwallbeschichtung, Schlitzbeschichtung, Zwillings-HSM-Beschichtung, Filmpressenbeschichtung, Größenpressenbeschichtung, Übertragungsfilmverfahren, Offset-Drucken, Tintenstrahldrucken, Laserdrucken, xerographischem Drucken, Rasterdrucken, flexographischem Drucken, kontinuierlichem Tintenstrahl, Flüssigtoner-Drucken, Heißfolienblockieren, insbesondere Rasterdrucken, Flüssigtoner-Drucken und Offset-Drucken ausgewählt ist.

17. Verfahren zum Produzieren eines Produkts gemäß Anspruch 13, umfassend das Ausführen der Schritte des Prozesses gemäß Anspruch 14 bis 16, wobei zusätzlich eine Klebstoffschicht auf die Beschichtungsschicht oder auf die weiße Druckfarbenschicht und/oder eine Oberfläche eines Papier-, Karton- oder Pappartikels derart angewendet ist, dass das transluzente oder transparente Papier und der Papier-, Karton- oder Pappartikel verklebt sind.

18. Verwendung des transluzenten oder transparenten Papiers gemäß Anspruch 1 bis 17 für Verpackungen, insbesondere Luxusverpackungen, als transparentes oder transluzentes Schutzband, Tasche, Hülle oder Plastiklaminat-Ersatz/- Alternative, wobei die Verpackung optional heißversiegelt ist, wenn die Beschichtungsschicht des Papiers ein Vinyliden-Kopolymer oder -Homopolymer, insbesondere ein Vinylidenchlorid-Homopolymer (PVDC) umfasst.

## Revendications

1. Papier translucide ou transparent comprenant :
(i) un substrat fibreux ayant une face avant et une face arrière, le substrat fibreux comprenant des fibres de cellulose raffinées à plus de 40 °SR et l'indice d'opacité dudit substrat fibreux étant inférieur ou égal à 45 % mesuré conformément à la norme ISO 2471 ; et
(ii) une ou plusieurs couches de revêtement, en particulier, une ou deux couches de revêtement disposées sur la face avant dudit substrat fibreux, comprenant un matériau choisi dans un matériau conférant des propriétés de barrière à l'humidité et ayant une capacité de transparence lorsqu'il est fourni comme couche de revêtement sur ledit substrat fibreux et permettant au papier translucide ou transparent d'être repulpable, ledit matériau étant choisi dans le groupe comprenant ou consistant en un copolymère ou un homopolymère de chlorure de vinylidène, un copolymère ou un homopolymère de styrène, tel que le polymère de styrène 1,3-butadiène, un copolymère ou un homopolymère d'acrylique, un copolymère ou un homopolymère de polyester, ou une paraffine, telle que la cire de paraffine.

2. Papier translucide ou transparent selon la revendication 1, dans lequel une ou plusieurs couches de revêtement sont également disposées sur la face arrière du substrat fibreux.

3. Papier translucide ou transparent selon la revendication 1 ou 2 ayant au moins l'une des caractéristiques suivantes ou une combinaison de celles-ci : (i) une hygroexpansivité inférieure ou égale à 1 %, de préférence, inférieure ou égale à 0,5 %, et encore plus de préférence, inférieure ou égale à 0,25 %, lors d'un changement d'humidité relative (HR) de 15 % à 80 %, puis à 15 % en 8 heures, ou (ii) un taux de transmission de la vapeur d'eau inférieur ou égal à 20 g/m²/jour à 85 % d'HR différentielle et 23° C, ou inférieur ou égal à 10 g/m²/jour à 85 % d'HR différentielle et 23 °C, ou inférieur ou égal à 5 g/m²/jour à 85 % d'HR différentielle et 23 °C.

4. Papier translucide ou transparent selon l'une quelconque des revendications 1 à 3 ayant un indice d'opacité inférieur ou égal à 20 % mesuré selon la norme ISO 2471.

5. Papier translucide ou transparent selon l'une quelconque des revendications 1 à 4, dans lequel le substrat fibreux a un grammage compris entre 40 et 200 g/m², en particulier, entre 40 et 140 g/m², et de préférence, entre 40 et 90 g/m².

6. Papier translucide ou transparent selon l'une quelconque des revendications 1 à 5, dans lequel le substrat fibreux comprend des fibres de cellulose raffinées à 60 °SR ou au-dessus de 80 °SR.

7. Papier translucide ou transparent selon l'une quelconque des revendications 1 à 6, dans lequel le substrat fibreux est un papier calque.

8. Papier translucide ou transparent selon l'une quelconque des revendications 1 à 7, dans lequel la ou les couches de revêtement totales sur une face du substrat fibreux a (ont) un poids de couche sèche dans une plage de 1 à 40 g/m², de préférence, de 2 à 20 g/m², encore plus de préférence, de 4 à 12 g/m².

9. Papier translucide ou transparent selon l'une quelconque des revendications 1 à 8, dans lequel au moins une couche de revêtement comprend un copolymère ou un homopolymère de chlorure de vinylidène, en particulier, un film de latex séché de copolymère de chlorure de vinylidène ou d'homopolymère de chlorure de vinylidène (PVDC).

10. Papier translucide ou transparent selon l'une quelconque des revendications 1 à 9, dans lequel une couche d'adhérence de l'encre est disposée sur la face arrière du substrat fibreux en l'absence d'une couche de revêtement, ou une couche d'adhérence de l'encre est disposée sur la face exposée de la ou des couche (s) de revêtement qui est / sont prévue(s) sur la face arrière du substrat fibreux, la couche d'adhérence de l'encre ayant une épaisseur dans une plage de 0,1 à 4 µm, en particulier, une couche d'adhérence de l'encre comprenant l'un quelconque des éléments suivants : acrylate de styrène, styrène-butadiène, acétate de polyvinyle, polyéthylène / acide acrylique ou amidon modifié, ou une combinaison de ceux-ci.

11. Papier translucide ou transparent selon l'une quelconque des revendications 1 à 10, dans lequel au moins une partie de la face exposée de la couche d'adhérence de l'encre ou de la face exposée de la couche de revêtement disposée sur la face arrière du substrat fibreux comprend une caractéristique imprimée, qui est inversée latéralement, de sorte que la caractéristique soit lisible depuis la face exposée de la couche de revêtement disposée sur la face avant du substrat fibreux et à travers le substrat fibreux.

12. Papier translucide ou transparent selon la revendication 11, dans lequel une ou plusieurs couches d'encre blanche est (sont) disposée(s) sur la caractéristique imprimée ou sur la totalité de la face arrière du substrat fibreux comprenant ladite caractéristique imprimée.

13. Produit comprenant un papier translucide ou transparent selon l'une quelconque des revendications 1 à 12, dans lequel le papier translucide ou transparent est collé sur un élément en papier, en carton ou en carte, avec une couche de colle ou d'adhésif disposée entre ledit élément en papier, en carton ou en carte et la ou les couches de revêtement ou la caractéristique imprimée ou la ou les couches d'encre blanche sur la face arrière du substrat fibreux, ladite colle ou ledit adhésif ayant une épaisseur dans une plage de 2 à 12 µm, en particulier, une colle ou un adhésif comprenant un matériau choisi dans les adhésifs polyuréthanes, les adhésifs acryliques, les adhésifs polychloroprènes à un ou deux composants, l'acétate de polyvinyle, l'amidon modifié, la méthylcellulose, la dispersion vinylique.

14. Procédé de production d'un papier translucide ou transparent selon l'une quelconque des revendications 1 à 13, comprenant les étapes consistant à :
a) fournir ou produire un substrat fibreux ayant une face avant et une face arrière, dans lequel le substrat fibreux comprenant des fibres de cellulose raffinées à plus de 40 °SR et l'indice d'opacité dudit substrat fibreux est inférieur ou égal à 45 % mesuré conformément à la norme ISO 2471 ;
b) appliquer une composition de revêtement sur la face avant du substrat fibreux, la composition de revêtement comprenant un matériau choisi dans un matériau conférant des propriétés de barrière à l'humidité et ayant une capacité de transparence lorsqu'il est fourni comme couche de revêtement sur ledit substrat fibreux et permettant au papier translucide ou transparent d'être repulpable, ledit matériau étant choisi dans le groupe comprenant ou consistant en un copolymère ou homopolymère de chlorure de vinylidène, tel qu'une dispersion aqueuse dudit copolymère ou comopolymère de chlorure de vinylidène, copolymère ou homopolymère de styrène, tel qu'une dispersion aqueuse de copolymère ou homopolymère de styrène, tel que styrène 1,3-butadiène, copolymère ou homopolymère d'acrylique, copolymère ou homopolymère de polyester, en particulier, polyester à base d'eau, ou paraffine, tel(le) que la cire de paraffine ;
c) sécher la composition de revêtement à une température comprise entre 70 et 200 °C pendant 0,2 à 1 minute, de manière à former une couche de revêtement ayant une épaisseur comprise entre 1 et 40 µm, de préférence, entre 2 et 20 µm, encore plus de préférence, entre 4 et 12 µm ;
d) répéter éventuellement les étapes b) et c) au moins une fois ; et
e) facultativement, appliquer et sécher également ladite composition de revêtement sur la face arrière du substrat fibreux au moins une fois, et / ou appliquer et sécher une composition pour une couche d'adhérence de l'encre sur la face arrière du substrat fibreux ou sur la ou les couche (s) de revêtement disposée(s) sur la face arrière,
en particulier, dans lequel ladite composition de revêtement et une composition pour une couche d'adhérence de l'encre sont appliquées par une technique choisie dans le revêtement de rouleau à rouleau, le couchage à la lame, le revêtement par pulvérisation, le revêtement à tige de Mayer, l'enduction par lame d'air, l'héliogravure directe, l'héliogravure offset, l'héliogravure inverse, le revêtement profond, le revêtement par rouleau lisse, le couchage rideau, le revêtement en cordon, le revêtement par fente, le revêtement HSM double, le revêtement de presse à film, le revêtement par presse encolleuse, et / ou le procédé de film de transfert, en particulier, l'enduction par lame d'air ou le revêtement d'héliogravure inverse.

15. Procédé selon la revendication 14, dans lequel une caractéristique est imprimée sur la face exposée de la couche d'adhérence de l'encre ou sur la face exposée de la couche de revêtement disposée sur la face arrière du substrat fibreux en mode inverse ou miroir (c'est-à-dire, inversion gauche / droite) par une technique choisie dans l'impression offset, l'impression à jet d'encre, l'impression laser, l'impression xérographique, l'impression sérigraphique, l'impression flexographique, l'impression à jet d'encre continu, l'impression à toner liquide, la typographie, la gravure laser et / ou le blocage de film à chaud, en particulier, l'impression offset, l'impression à jet d'encre, l'impression sérigraphique, l'impression à jet d'encre continu, l'impression à toner liquide.

16. Procédé selon la revendication 15, dans lequel une ou plusieurs couches d'encre blanche est (sont) appliquées sur la caractéristique imprimée par une technique choisie dans le revêtement de rouleau à rouleau, le couchage à la lame, le revêtement par pulvérisation, le revêtement à tige de Mayer, l'enduction par lame d'air, l'héliogravure directe, l'héliogravure offset, l'héliogravure inverse, le revêtement profond, le revêtement par rouleau lisse, le couchage rideau, le revêtement en cordon, le revêtement par fente, le revêtement HSM double, le revêtement de presse à film, le revêtement par presse encolleuse, le procédé de film de transfert, l'impression offset, l'impression à jet d'encre, l'impression laser, l'impression xérographique, l'impression sérigraphique, l'impression flexographique, l'impression à jet d'encre continu, l'impression à toner liquide, la typographie, le blocage de film à chaud, en particulier, l'impression sérigraphique, l'impression à toner liquide, et l'impression offset.

17. Procédé de fabrication d'un produit selon la revendication 13, comprenant la mise en œuvre des étapes du procédé selon les revendications 14 à 16, dans lequel, en outre, une couche de colle est appliquée sur la couche de revêtement ou sur la couche d'encre blanche et / ou une surface d'un élément en papier, en carton ou en carte, de manière à coller le papier translucide ou transparent et l'élément en papier, en carton ou en carte.

18. Utilisation du papier translucide ou transparent selon les revendications 1 à 17 pour l'emballage, en particulier, l'emballage de luxe, en tant que ruban pochette, emballage ou remplacement / alternative de stratifié plastique protecteur transparent ou translucide, dans laquelle l'emballage est éventuellement thermoscellé lorsque la couche de revêtement du papier comprend un copolymère ou un homopolymère de chlorure de vinylidène, en particulier, un homopolymère de chlorure de vinylidène (PVDC).
